

April 25, 1961

W. H. STICKNEY ET AL

2,981,330

PULP MOLDING DIE

Filed Dec. 20, 1956

3 Sheets-Sheet 1

FIG. 1



FIG. 2



INVENTORS

Wendell H. Stickney  
Richard F. Reifers

BY

KARL W. FLOCKS  
ATTORNEY

April 25, 1961

W. H. STICKNEY ET AL

2,981,330

PULP MOLDING DIE

Filed Dec. 20, 1956

3 Sheets-Sheet 2

FIG. 3



FIG. 4



FIG. 5



INVENTORS  
Wendell H. Stickney  
Richard F. Reifers

BY

Karl W. Flocks

ATTORNEY

April 25, 1961

W. H. STICKNEY ET AL

2,981,330

PULP MOLDING DIE

Filed Dec. 20, 1956

3 Sheets-Sheet 3

FIG. 6



FIG. 7



INVENTORS

Wendell H. Stickney  
Richard F. Reifers

BY

KARL W. FLOCKS  
ATTORNEY

1

2,981,330

## PULP MOLDING DIE

Wendell H. Stickney, Wilbraham, Mass., and Richard F. Reifers, Lincolnwood, Ill., assignors to Diamond National Corporation, a corporation of Delaware

Filed Dec. 20, 1956, Ser. No. 629,495

9 Claims. (Cl. 162—411)

The present invention relates to a pulp molding die and more particularly to a porous die suitable for use in producing pulp articles and the method of making the die.

Heretofore, pulp molding dies have been made with a woven wire cloth material stretched to conform to the die surface. The manufacture of this type of die has caused many difficulties due to the limited amount of distortion or stretching of which the wire cloth is capable to enable it to conform to the die surface. When the distortion of the woven wire is too great, it either tears or ruptures, or the mesh becomes so distorted as to cause it to fail to function properly as a pulp molding surface. This difficulty is particularly prevalent in the manufacture of dies for the making of pulp articles such as egg cartons and other complex designs.

It is therefore an object of the present invention to provide a novel pulp molding die that can be readily manufactured to conform to any desired design.

It is further object of the present invention to provide a novel pulp molding die that is made up of a porous sintered material molded to the desired design.

Another object of the present invention is to provide a novel pulp molding die that is made up without wire woven cloth applied thereto.

A still further object of the present invention is to provide a novel pulp molding die that is simple in construction and results in a molded article of improved appearance.

These and other objects and the nature and advantages of the instant invention will be apparent from the following description taken in conjunction with the accompanying drawings, wherein:

Fig. 1 is a perspective view of a pulp molding die in accordance with the present invention;

Fig. 2 is a perspective view of the die with the contoured molding surface removed;

Fig. 3 is a perspective view of the metal plate and attached reinforcing structure in inverted position over the male master pattern prior to application of the resin coated spherical particles;

Fig. 4 is a perspective view of the die shown in Fig. 1 in inverted position;

Fig. 5 is a sectional view taken along the line 5—5 of Fig. 1;

Fig. 6 is a perspective view of the male master pattern; and

Fig. 7 is a top plan view of an article molded from the die of Fig. 1.

Molding dies of the type disclosed herein are used to form or mold pulp articles from liquid pulp mixtures, these mixtures being composed of fibers and some liquid, such as water, the liquid being drawn through the die, leaving a layer or coating of felted fibers on the molding surface. The article so formed is then removed from the molding surface and the process is repeated. The operation of pulp molding dies is a well understood art,

2

and it is believed unnecessary to discuss their functions in greater detail.

The following description of the molding die and the method of making it is described in conjunction with the molding of an egg carton having therein a plurality of pocket sections with a cover portion connected to this pocket section by a hinge structure which will enable it to be folded over, forming a closed container. This egg carton is illustrated in Fig. 7 and comprises a cellular 10 compartmented bottom section, generally designated 10, to which a non-cellular or open faced, tray-like cover section 11 is integrally hinged by a longitudinal crease 12 at corresponding side margins of the section. Cover section 11 has pairs of opposed end walls 13 and side walls 14 integrally joined by rounded corners 15, and a flat top panel 16 is likewise integrally joined about its periphery with the walls. The exterior surface of this panel is smooth and continuous, suitable for the reception of printed matter or ornamentation.

20 The cover section side walls are of scalloped shape featuring longitudinally spaced, outwardly curved or recessed bays 17 to increase the egg room in the cover section, which recesses are spaced by intervening, inwardly extending abutment portions 18. These portions come 25 into contact with the cellular bottom section 10 when the carton is closed.

The interior of bottom section 10 is partially subdivided into two rows of six egg receiving cells 19, by a longitudinally extending series of upstanding center separator 30 posts 20 which are of generally rectangular outline at their tops.

An elongated internal cover bracing and locking flange 26 is integrally hinged by a longitudinally extending crease 27 to the side margin of bottom section 10 35 opposite its cover hinge 12. Flange 26, like the side walls of cover section 11, is of generally scalloped outline. It has egg accommodating bays or recesses 28 which are in transverse alignment with bottom section egg cells 19. The locking means comprises a pair of 40 locking elements or lugs 30 which are integrally molded in the flange 26 to project outwardly adjacent the free outer edge thereof, and detent apertures 31 molded in the front wall 14 immediately adjacent its junction with cover top panel 16.

45 In use, when the eggs have been deposited in the bottom cells 19, flange 26 is swung to upstanding position adjacent the front row of eggs and the cover section 11 is swung downwardly into externally telescoped relation over the flange. As this occurs, the free front cover wall 50 14 slides downwardly over the locking lugs 30 until the flange and cover are in interlocked relationship.

The die, in accordance with the present invention, is used for molding the egg carton described heretofore.

The die shown in Fig. 1, designated in its entirety by 55 the numeral 40, includes a flat metal plate 42 prepared with a window opening 44 on the center thereof corresponding in shape to the outer periphery of the egg carton. A plurality of holes 45 are provided in the plate 42 for attaching the finished die to a conventional die 60 box. The plate 42 becomes effective in use as a margin strap and also as a support for the contoured molding surface. Attached to the underside of the plate 42 is a reinforcing structure or grid arrangement which may consist of a plurality of rods 46 supported at each end 65 in a plate 48, each of which is attached to the plate 42 by screws. A plurality of pedestal supports 50 are arranged on the rods at equal intervals, each of which has a plurality of feet 52. Four feet 52 are illustrated on each support 50. The supports act to absorb any tendency for the molding die to collapse under vacuum. The feet 52 rest on the platen of the main wet end cylinder 70 of the molding apparatus.

To form the contoured molding surface of the die, a male master mold or platter 54 is utilized. This master mold or pattern 54 is illustrated in Figs. 3 and 6. This mold or pattern may be made of plaster or metal and conforms to the shape of the article to be molded when in the flat position.

To make the desired pulp molding die 40, the metal plate 42 with its attached grid arrangement is inverted and placed over said male master mold or pattern 54 so that the window opening 44 in the plate is positioned to fit over the periphery of the pattern 54 with the contours in the pattern extending upwardly through the window opening 44 between the rods 46 and the pedestal supports 50 of the grid arrangement, as shown in Fig. 3. Side plates 56 are attached at each side to the plates 48, whereby the entire pattern is enclosed.

For ease in removal after the molding of the die, the male master or pattern 54 may be coated with a silicone resin and baked. The silicone acts as a release agent during the molding.

The molding material 58, which has been previously prepared, is poured over the pattern 54 until the pattern is completely covered and the molding material reaches the height of the plates 48 and 56, as shown in Fig. 4. The entire mold is vibrated during the pouring of the molding material.

The molding material 58 is made up of a plurality of small spherical particles having a diameter of approximately 3 to 50 mils, preferably in the range of 8-30 mils. These particles may be small glass beads which are spheres of an approximate diameter of 15 mils, metal powders which are spherical particles of a diameter of 15 to 25 mils, spherical sand particles of similar diameter or other spherical particles. The spherical particles are coated with a phenolic resin and dried to yield a freely pourable coated powder.

After the coated spherical particles have been poured into the mold and vibrated sufficiently to fill all crevices, the mold is placed in an oven and heated to a temperature of about 350° F. for several hours. After cooling to room temperature, the resulting die is removed from the pattern 54. This die, which is illustrated in Fig. 1, has a porous resin-sintered spherical particle structure wherein the spherical particles are bonded together at portions of their peripheries by the cured resin leaving voids and pores for the passage of liquid during the pulp molding operation.

A specific example of the treatment of the spherical particles and the molding and curing of a die is as follows: One hundred parts by weight of spherical glass beads having a diameter of .015 inch are placed in a mixer and a mulling mix action is started. Slowly three-fourths part by weight of a liquid phenol-formaldehyde bonding resin is added to the mixer. When the mixture is complete four parts by weight of a dry powdered phenol-formaldehyde resin are added slowly until the mixture has become complete and uniform. The resulting coated beads should be dry enough to pour freely. The coated particles are now poured into the mold as illustrated in Figs. 3 and 4, while vibrating the entire mold. The pattern has previously been treated with a silicone and baked to provide a release agent. The mold is placed in an oven and the resin is cured by heating at 150° for two hours. The temperature is increased in increments of 20° F. for ten hours until a temperature of 350° F. is reached. The temperature is held at 350° F. for two hours. The mold is removed from the oven and allowed to cool to room temperature. The die is now removed from the pattern and is ready for use in pulp molding.

A second example of this method is as follows: 2000 cc. of bronze powder, approximately spherical in shape and about .018 inch in diameter was placed into a muller mixer. The composition of the metal powder is not critical, however the bronze powder used here contained 95.5% copper coated with 4.5% tin. 30 cc. of alcohol

was added to the mixer and the mixing continued for two minutes. With the mixer running 68 gms. of a liquid phenol-formaldehyde bonding resin was very slowly added until the mixture was complete, about eight minutes.

5 Each particle should be coated with the liquid, and the resulting powder should spill freely without balling up. With the mixer still running, 204 gms. of a dry powdered phenol-formaldehyde resin was added gradually, and mixing continued for about eight minutes. The treated powder was now ready for pouring freely into the mold, and the mold could be vibrated or rapped with a hammer to pack the particles into all crevices. It was now ready for curing to produce the finished mold. The mold was heated to 340° F. for three hours. After removal of the die from the mold, the die was returned to the oven for another three hours.

If desired, the die 40 may consist of a "window plate" 42 which is attached directly to a rectangular die box (not illustrated). Various forms of reinforcing can be 10 utilized in the die box, such as reinforcing rods buried in the resin-sintered mass, and a rectangular piece of expanded metal grid added to the surface of the mass to add structural strength. Likewise, when desired, the spherical particles may extend flush with the surface of the "window plate" 42 and margin straps may be assembled onto the plate to form the outline of the egg carton to the thickness desired. This marginal thickness in the "window plate" 42 is illustrated at 41 in Fig. 1.

The finished die assembly 40 is now ready for molding cartons. A typical pulp furnish that may be used is

|     |                            |
|-----|----------------------------|
| 75% | 85% blank news             |
|     | 15% bleached kraft         |
| 25% | 90% newspaper              |
|     | 10% bleached kraft deinked |

The consistency is 60%, molding time 7 seconds, utilizing a vacuum before molding of 5" Hg and 18" Hg after molding. A transfer air pressure of 50 p.s.i. is used and the cartons are dried on a plaster drying form in an oven at 350° F. for twenty-five minutes.

The curing time recited heretofore for sintering the resin and spherical particles is a function of the weight and cross-section of the article being formed, and should be varied accordingly.

45 The proportions of resin to spherical particles should be maintained such that the resulting material is as rich in resin as possible and yet capable of freely flowing like dry sand. Various types of spherical particles may be utilized as well as various types of bonding agents.

50 This method of preparing dies has many advantages over the presently used method utilizing wire woven cloth. Experimental and pilot plant work can be accomplished with much less time and expense where it is necessary to study design changes and modify the molding die accordingly. Screenless dies, in accordance with the present invention, are easily reconstructed in different dimensions with altered design features incorporated. Temporary molding dies may be quickly and cheaply prepared where only a few product samples are required.

55 The screenless molding dies in accordance with the present invention may be made at less than half the expense of conventional screened molds. Maintenance of screenless molding dies described in this application is simplified. When a unit becomes damaged it may be scrapped and incur less expense than an overhaul of a conventional screened molding die. The appearance of the product made on a screenless molding die in accordance with this invention would be noticeably improved. The surface of the product is uniform and bears no marks of the screens or the seams.

60 It will be obvious to those skilled in the art that various changes may be made without departing from the spirit of the invention and therefore the invention is not limited to what is shown in the drawings and described in the specification but only as indicated in the appended claims.

## What is claimed is:

1. A pulp molding die having an exterior, open-faced, contoured molding surface provided with a peripheral portion, said molding surface comprising a porous structure of a plurality of small spherical bodies sintered together by a phenolic resin, said spherical bodies having a diameter of approximately 3 to 50 mils and being made of a material which is hard, non-porous and stable at the curing temperatures of said phenolic resin.

2. A pulp molding die in accordance with claim 1, wherein said molding surface is reinforced by a metal grid arrangement embedded therein.

3. A pulp molding die in accordance with claim 1, wherein said spherical bodies are glass beads.

4. A pulp molding die in accordance with claim 1, wherein said spherical bodies are metal.

5. A pulp molding die having an exterior open-faced, contoured molding surface provided with a peripheral portion, said die comprising a flat metal plate, a window opening in said plate in which said molding surface is located, said opening corresponding to the peripheral portion of said molding surface, said molding surface comprising a porous structure of a plurality of small spherical bodies sintered together by a phenolic resin, said spherical bodies having a diameter of approximately 3 to 50 mils and being made of a material which is hard, non-porous and stable at the curing temperatures of said phenolic resin.

6. A pulp molding die in accordance with claim 5, wherein a reinforcement structure is embedded in said molding surface, said reinforcement structure being attached to said metal plate.

7. A pulp molding die in accordance with claim 5, wherein said spherical bodies are glass beads.

8. A pulp molding die in accordance with claim 5, wherein said spherical bodies are metal.

5 9. A pulp molding die having an exterior open faced contoured molding surface provided with a peripheral portion, said die comprising a flat metal plate, a window opening in said plate conforming to the shape of the peripheral portion of the desired molding surface, a grid arrangement located below said window opening, a molding surface located in said window opening the upper surface of said molding surface being located below the upper surface of said metal plate, said molding surface having an upper surface of the desired configuration and a thickness sufficient to embed said grid arrangement therein, said molding surface comprising a porous structure of a plurality of small spherical bodies sintered together by a phenolic resin, said spherical bodies having a diameter of approximately 3 to 50 mils and being made of a material which is hard, non-porous and stable at the curing temperatures of said phenolic resin.

## References Cited in the file of this patent

## UNITED STATES PATENTS

|           |         |                |
|-----------|---------|----------------|
| 1,669,426 | Shaw    | May 15, 1928   |
| 1,742,411 | Muller  | Jan. 7, 1930   |
| 2,079,667 | Swift   | May 11, 1937   |
| 2,273,055 | Manson  | Feb. 17, 1942  |
| 2,392,804 | Basolo  | Jan. 15, 1946  |
| 2,400,091 | Alfthan | May 14, 1946   |
| 2,619,012 | Brennan | Nov. 25, 1952  |
| 2,718,826 | Lambert | Sept. 27, 1955 |
| 2,750,632 | Kish    | June 19, 1956  |
| 2,851,931 | Leitzel | Sept. 16, 1958 |

## FOREIGN PATENTS

|               |         |               |
|---------------|---------|---------------|
| Great Britain | 165,500 | June 27, 1921 |
| Australia     | 117,319 | July 27, 1943 |